

## UNITED STATES PATENT OFFICE

2,170,814

## METHOD OF PREPARING COPPER POWDER

Joseph E. Drapeau, Jr., Calumet City, Ill., assignor  
to The Glidden Company, Cleveland, Ohio, a  
corporation of Ohio

No Drawing. Application December 6, 1937,  
Serial No. 178,347

2 Claims. (CL 75—72)

This invention relates to the production of copper powder, and has particular reference to a new form of pure copper powder, which combines low apparent density, a porous structure under the microscope, and a good degree of resistance to atmospheric influences. It further relates to a process for producing this new copper powder.

Powdered copper is a raw material that is used extensively in several industries, including the paint, electrical and bearing industries. In the paint field, color and "leafing" properties in paint vehicles are important; in the electrical field, conductivity, and mechanical strength of molded products made from the powder, are the prime considerations; while in the bearing field, mechanical strength of the bearings produced is, of course, by far the most important property. In all cases, maximum resistance to atmospheric corrosion is likewise desirable.

20 Copper powder has been produced by the electrical method, which consists of electrolytic deposition, employing current densities (cathodic) between 50 and 150 amperes per square inch of cathode deposition surface, in the presence of suitable addition reagents (colloids), causing the copper to be plated out of solution in a loose, sponge-like mass. This sponge-like copper product is washed as free as possible of the electrolyte solution and dried under non-oxidizing conditions. The outstanding disadvantage of this type of copper powder is its high cost, and its marked tendency to reoxidize when exposed to atmospheric conditions. The traces of electrolyte salts increase the rate of oxidation of the copper powder.

Another method of making copper powder has been to stamp it out of thin sheets of copper alloy metal, using a lubricant. The resultant powder, when examined under the microscope, is in the form of flat sheets, coated with lubricant. While excellent color and leafing are obtained in paint vehicles, the lubricant results in poor mechanical strength and electrical conductivity. Such flake powder is dense, has no mobility, does not weld, and is not suitable for bearings, and only in special cases for brushes. The excellent color is due to the alloying of small percentages of zinc or aluminum with copper.

It has also been proposed to obtain copper powder by reducing cupric or cuprous oxide powder, in a furnace, by the use of various reducing gases. The process may be carried out on the furnace hearth, or in trays. The mass that is removed from the furnace in the form of sintered lumps or cakes, is then broken up by milling. The resultant powder has an apparent gravity ranging from just above 2.5 up to 3.0 and higher; under the microscope, it gives the appearance of solid nodules. It has fair electrical conduc-

tivity, and may be used in bearings with fair results.

According to the present invention, a process is provided whereby a new form of copper powder is produced having superior properties as to electrical conductivity and mechanical strength, and is characterized by its low apparent gravity (below 2.5 grams per c. c.), its porous structure under a microscope, and its ability to withstand atmospheric conditions without blackening.

The invention comprises the conversion of copper wire or other pieces of copper metal such as punchings, shot, etc., into copper powder. The steps comprise first, oxidizing the copper to copper oxide, preferably cuprous oxide, breaking up this oxide, and then reducing the powdered oxide to copper. By this procedure, a pyrometallurgical method is provided for the production of copper powder from copper, which powder has the properties and advantages enumerated above.

My process comprises first, roasting of pieces of copper, of uniform cross-section, continuing the roasting to the point where the bulk of the copper has been oxidized, but there still remains a core of metal. An oxidizing atmosphere is maintained, and I have found that the presence of water vapor accelerates the reaction. The charge is pulled, and allowed to cool in air; a thin film of cupric oxide forms on the surface only. The oxide is separated from the metal core by grinding in a rod or ball mill, and screening or air classifying. The resultant product is a cuprous oxide which contains 2% or less of cupric, and at least 98% of cuprous oxide. The temperature is preferably between 800° and 1780° F., as at these temperatures cuprous oxide is formed.

As an example, a charge of 2,000 pounds of 10 gauge pure copper wire was placed in a hand rabbled furnace, and heated at 1650° F. in an oxidizing atmosphere in the presence of water vapor for 48 hours. The charge was rabbled from time to time. A 79.0% conversion to cuprous oxide was obtained, after separation of the oxide from the metal core.

Using the same charge, without adding water vapor, the same percentage conversion took 68 hours.

The charge is drawn from the furnace, and cooled in air. A thin film of cupric oxide forms on the surface of the pieces; but this film prevents oxidation below it. The cooled charge is then ground, preferably in a rod or ball mill; the oxide is powdery, the metal malleable, so that separation is easily effected. The metal may be screened out, or the mixture may be air classified. The resultant powdered cuprous oxide is 98% or more pure; the impurity is largely the film of cupric oxide formed during cooling.

The oxide powder, which is substantially free

- from any occluded salts, is then subjected to a reducing action. For most economical results, it is preferred to use a cuprous oxide powder which is substantially pure, as it has only half as much oxygen to remove as cupric oxide. However, it will be understood by those skilled in the art, that a copper oxide powder containing varying proportions of cuprous and cupric oxide may be used in the reduction. The important thing to be kept in mind is that the oxide be free of occluded salts, and it is preferable that the oxide be substantially a pure, uniform cuprous oxide, as will be produced by the above described oxidation of copper wire, etc.
- 15 The reduction and heating of the oxide is conducted in a furnace, and I may use any of the common reducing gases—hydrogen, carbon monoxide, artificial or natural illuminating gas, methane, ethylene, etc.
- 20 Temperatures may vary over a considerable range. Below 350° F., the reaction proceeds too slowly to be economically feasible; and in no case should the temperature exceed 700° F., at which point the materials tend to sinter. However, much superior results as to low apparent density are obtained by keeping the temperature at a minimum; and I prefer to operate in the range of 350–500° F. for optimum results. Higher temperatures may be used, up to 700° F.; but as the temperature increases, the apparent density likewise increases.

An important feature of my process is the continuous motion imparted to the powder during the reducing, whereby the tendency to sinter is minimized. While any method of rabbling may be used which keeps the particles broken up, it is of course necessary that air be excluded. A rotating drum, provided with attached rabbles, provides the most simple, effective apparatus for the purpose. A mechanical rabbler, on a furnace bed designed to exclude air, might do as well, as continuous rabbling is not essential to good results, although frequent rabbling is; but such a rabbler is much more difficult to operate than a rotating drum.

In place of the attached rabbles, I have obtained satisfactory results by the use of irregular shaped light weight metal pieces in the drum. In this connection, it is important that any milling action in the drum be minimized, as such action increases apparent density and reduces porosity; and the rabbling must be carried out in a manner which will not at the same time introduce a ball or hammer milling effect.

55 Another important item in regard to this step of the process is the time required for reduction. The reaction should preferably be carried on rapidly, in order to reduce the milling action due to the attrition of the particles on each other. Reaction times of over 18 hours should be avoided where low density is desired.

After the oxide powder has all been reduced, the powder is allowed to cool in a reducing atmosphere until room temperature is reached, in order to prevent reoxidation of the copper. This is most easily accomplished by sealing up the drum containing the copper powder and reducing gases from the air until the powder has cooled to approximately room temperature.

70 The cooled copper powder may then be treated in a ball mill or other mill to break up the agglomerated material.

The product obtained by the process as outlined differs from conventional prior art copper powders in many important respects. In the

first place, the particles exhibit a porous structure under the microscope, in distinction from the sheet structure of stamped powder, the nodule structure of the prior art reduced powder of the type previously referred to and the dendritic structure of electrolytic powder.

A second distinction lies in its range of particle size. The nodule powder of the prior art will weigh, in all cases, more than 2.5 grams per c. c., and may range up to 3.5; my powders run below 2.5 in apparent density, and ordinarily will run about 2.0, although with extreme care they may be kept below 2.0. For powder of 100 mesh or finer, particle size seems to have no effect on apparent density. The electrolytic coppers may be made in apparent density of from 0.5 to 2.0, while the flaked stamped powders may vary from 1.0 to 3.5; these apparent densities, however, depend largely on particle size, and on the distribution of the various sizes of particle in the mass.

15 A third distinction lies in the ability of my products to withstand atmospheric corrosion. Ordinary electrolytic copper powder will be substantially black after 60 days exposure to the air, while my powder retains its color. It is true that both stamped and nodule powders will retain their color; but the stamped product is coated with lubricant, and the nodule powder has decidedly less reactive surface as compared with my porous powders.

25 In the electrical field, my powder gives results superior to prior art powders. When incorporated into brushes by mixing with carbon or graphite, tests indicate that equivalent conductivity and strength may be obtained by using approximately 10% less of my powder than prior art reduced powder. The brushes produced are softer, and produce less abrasive wear on commutators.

35 In the bearing field, the usefulness of my new powder is particularly apparent. Comparative tests were made, using my new powder and an ordinary prior art powder commonly used in the bearing industry. The following table shows the results obtained in a typical test run:

|                                                                                    | High density copper powder substantially non-porous | Low density copper powder substantially porous | 50    |
|------------------------------------------------------------------------------------|-----------------------------------------------------|------------------------------------------------|-------|
| Apparent density in gram per cubic centimeter                                      | 3.2                                                 | 2.00                                           | 55    |
| Flow or mobility relation (relative weight through standard orifice in given time) | 100                                                 | 87                                             |       |
| Screen analysis:                                                                   |                                                     |                                                |       |
| On 150 mesh                                                                        | do                                                  | 0.0                                            | 0.0   |
| On 325 mesh                                                                        | do                                                  | 45.0                                           | 46.0  |
| Through 325 mesh                                                                   | do                                                  | 55.0                                           | 54.0  |
| Sintering data:                                                                    |                                                     |                                                |       |
| Unsintered weight                                                                  | grams                                               | 14.53                                          | 14.56 |
| Unsintered length                                                                  | inches                                              | 0.679                                          | 0.688 |
| Unsintered width                                                                   | do                                                  | 0.818                                          | 0.817 |
| Sintered length                                                                    | do                                                  | 0.733                                          | 0.736 |
| Sintered width                                                                     | do                                                  | 0.839                                          | 0.833 |
| Radial strength                                                                    | lbs./sq. in.                                        | 147                                            | 189   |
| Radial strength ratio                                                              | percent                                             | 100                                            | 128.5 |
| Oil absorption                                                                     | percent by weight                                   | 3.42                                           | 3.87  |
| Oil absorption ratio                                                               | percent                                             | 100.0                                          | 110.4 |

The bearings were produced with a compression of the above weights of copper powder in dies at 50,000 # per-sq. in. pressure.

70 The process may be modified as described in the specification. For best results, optimum conditions should be maintained throughout; but it is possible to make fairly good copper powder.

even by disregarding temperatures, etc., to some extent.

By my method it is now possible to make for the first time a copper powder of porous structure with a large reactive surface, and with low apparent density, which at the same time will resist atmospheric corrosion. The copper powder of my process is a low cost product capable of replacing high cost electric copper powder in the bearing and electrical fields and having the added advantage of resistance to atmospheric corrosion and freedom from occluded salts.

This application is a continuation in part of applications Serial No. 729,443, filed June 7, 1934, and Serial No. 3,499, filed January 25, 1935.

15 I claim:

1. The method of producing copper powder which comprises roasting pieces of substantially pure copper presenting a large surface area to oxidation in an oxidizing atmosphere, to produce a surface oxidation to cuprous oxide, stopping the oxidation while a core of metal remains un-  
20 oxidized, to maintain the cuprous state of the

oxide, milling the copper oxide, separating the powdered oxide from the copper, and reducing the oxide to metallic copper by roasting in a reducing atmosphere at a temperature below that at which substantial sintering occurs.

2. The process of producing copper powder which comprises roasting pieces of substantially pure copper of substantially uniform cross section presenting a large surface area to oxidation in an oxidizing atmosphere at temperatures between 800° and 1780° F., to produce a surface oxidation of cuprous oxide, stopping the oxidation while a core of metallic copper remains un-  
10 oxidized, to maintain the cuprous state of the oxide, milling the resulting material to powder 15 the cuprous oxide, separating the cuprous oxide from the metallic copper core, and reducing the milled cuprous oxide by roasting in a reducing atmosphere at a temperature between 350° and 700° F., and cooling the reduced material in a 20 reducing atmosphere.

JOSEPH E. DRAPEAU, JR.